

## UNITED STATES PATENT OFFICE

ROBERT IRVING COWEN, OF NEW YORK, N. Y.

COLORED AND TINTED PARCHMENT PAPER AND THE LIKE AND PROCESS FOR THE  
MANUFACTURE OF THE SAME

No Drawing.

Application filed November 19, 1925. Serial No. 70,196.

Hitherto the manufacturers of parchment papers have not been able to produce satisfactory and reliable results in making tinted and colored parchment papers; they have 5 also been somewhat limited in the variety of colors which could be successfully applied to papers of this character; and, again, it has been found under present known methods that, in order to produce deeper shades of 10 color with dyes, large excess of the amounts necessary to produce the desired coloring will have to be used in the processes, involving considerable loss in dyestuffs.

As is generally known, parchment paper is 15 made by passing unsized paper through a parchmentizing bath, for instance, sulphuric acid, and then through a clear water bath in order thoroughly to wash the paper free from excess of the acid. By this treatment a sur- 20 face film of "amyloid" is formed upon both sides of the paper and around each fiber, the thickness of such film depending principally upon the time of immersion of such unsized paper in the acid bath, the temperature of 25 the bath, the texture of the paper, etc. This amyloid film or coating produces so-called "parchment" paper or "vegetable parchment." In the process heretofore employed for the 30 production of colored papers of this character, the tint or color is incorporated in the beaters, or applied to the web by a print roll before or after going through the calenders as stated; by this process the result is not always satisfactory, and the depth of 35 shade and the number of colors which can be specially utilized is limited.

If colored parchment paper is to be made by adding the dyestuff to the beaters, the manufacturer is limited as to the dyestuffs he 40 can use for the following reasons. Acid and direct dyes cannot be used without a mordant, as they will not attach themselves to the fibers with any permanency and will mostly be washed out in the "white water" when the 45 beaten stock is run on to the wire. If a mordant, such as rosin size or alum, or a combination of the two is used, the paper will not parchmentize properly or at all when it is run through the parchmentizing bath. Thus 50 acid and direct dyes cannot be used satis-

factorily for coloring the paper in the beaters. However, basic dyes will attach themselves to the fibers without the use of a mordant, although some will naturally be lost in the white water. On the other hand, many 55 basic dyes will be destroyed or decolorized when the paper is put into the parchmentizing bath, or dissolved by it. On subsequent washing out of the acid the concentration of dye left in the paper would be too small to 60 color it satisfactorily.

I have found that papers of this class can be produced so as to enable the manufacturer to employ a wider range of colors and to do this more economically and more satisfac- 65 torily by my process than has been possible to do with the existing methods, and it is also possible to produce, for instance, a black parchment paper of highly satisfactory quality and which hitherto has not been made sat- 70 isfactorily. For instance, I am able, with my process, to produce yellow, orange, pink, blue, green, purple and black, or any other color, shade or tint of a high degree of per- 75 fection.

By my process the dyestuffs or coloring materials are so applied that they become incorporated in the amyloid film, which forms on the paper, or rather around the fibers of the paper, thus treated. Instead of applying 80 the dyestuffs in the beaters for the purpose of coloring the pulp from which the paper is to be manufactured, I apply the coloring matter in the acid bath which is used for giving the paper its amyloid coating. I have found 85 that there are several types of coal-tar dyes especially which will do the work very satis- factorily in the manner indicated.

On adding an organic dye to concentrated 90 sulphuric acid, say of about seventy-five per- cent strength, it may be, depending upon the character of the dye, (1) left unchanged chemically; (2) it may be changed to some other color, and upon subsequent dilution, 95 that color may disappear and the original color return; (3) it may be changed to a different color, and that color may remain on dilution; (4) the dye may be entirely decom- posed and be useless for further operaton; or, 100

again, (5) the dye may not dissolve in the acid solution at all.

The organic acid dyes, or most of them at least, are soluble in sulphuric acid, and, although some of these change in color or shade through the action of the acid or may give a colorless or nearly colorless parchmentizing bath, the original color reappears upon passing the treated paper through the water bath for washing out the excess of acid, and the paper is found to have been colored in a very satisfactory manner.

This class of acid dyes is mainly soluble in water, but, after the treatment in the manner indicated, the dye, being incorporated in the amyloid film itself, washes out very little in the subsequent treatment of the water bath which is used to wash out the excess of acid. Obviously any dye which is chemically decomposed entirely by the acid is not serviceable.

I have also found that dyes which are insoluble in the acid bath may be used if they are present in fine suspension. For instance, when I use National Erie fast scarlet (color index No. 326) in such a suspension in the acid bath, the paper presents the same color as the plain parchment, but, when the paper is subsequently washed in a diluting bath, the dye begins to dissolve and colors the paper quite satisfactorily.

As an illustration of some of my experiences with various organic dyes of different classes and the results to be obtained therewith, I may state at this point that chinoline yellow (color index No. 801) produces a yellow dye bath and produces a fine yellow color in the paper; auramine O concentrated (color index No. 655) gives a colorless acid bath, but the color develops again on washing and produces a good dyeing effect; orange A (color index No. 151) produces a red dye bath, but gives a good orange color to the paper after washing; croceine scarlet C (color index No. 252) produces a purple acid bath, but gives a good scarlet color in the finished paper; National Erie fast scarlet, which is insoluble in the acid solution and must therefore be suspended therein, produces a satisfactory color after passing through the wash bath; acid scarlet 3 R (color index No. 196) dissolves in the acid bath to a wine-red color and gives a good red shade in the finished paper; acid blue R (color index No. 672) dissolves in the acid bath with a brownish-green color that gives a good blue color effect in the paper; acid blue C F (color index No. 671) dissolves in the acid with a blue color and gives the same effect in the paper after treatment; acid violet 4 B N S (color index No. 695) dissolves in the acid bath with a yellow color and dyes the paper purple after passing through the wash bath; acid green double (color index No. 666) dissolves with a yellowish-brown color but gives a good

green coloring effect in the paper; and similarly naphthylamine black D (color index No. 308) produces a blue-black solution and produces a good black finished paper.

On the other hand, I found some dyes, as, for example, pontamine yellow (color index No. 365), and polar red B concentrated (color index No. 430) are permanently destroyed by the acid and can therefore not be used for the purpose stated.

In general, therefore, it will be seen that the paper produced by this process affords a wide range of color; that the dyes are incorporated in the amyloid film; that the shade of color can be readily controlled by the amount and character of the dye put into the acid bath, which cannot be so well and conveniently done when the coloring matter is introduced into the beaters. Obviously the amount of dye depends upon the nature of the dye itself and the depth of color which it is desired to obtain, and will vary considerably, ranging from, say, a fraction of an ounce to several ounces per pound of acid.

To illustrate the further detail my manner of producing this improved colored "parchment" paper or "vegetable parchment", I give the following examples of the manner in which the process is employed, wherein it will be noted that the process is modified somewhat according to the nature of the dye in its relation to the acid bath:

1. *Dye soluble in water and in acid giving colored dye-bath.*—From one one-hundredth of an ounce to ten ounces of chinoline yellow (color index No. 801), or some similar dye, depending on the shade desired, is thoroughly dissolved in the parchmentizing acid bath, the above amount being added per pound of acid in the bath. The paper is run through the bath in the usual manner and washed in the usual manner, the resulting parchment being dyed a light, pale, or deep shade of yellow, according to the amount of the dye added to the bath.

2. *Dye soluble in water and in acid giving colorless dye-bath.*—From one one-hundredth to ten ounces of auramine O (color index No. 655) or similar dye, depending on the shade desired, is dissolved in the parchmentizing bath per pound of acid, and which, in this case, gives a colorless bath. The paper is passed through the bath in the usual manner. On going into the washing bath of water, the color develops as the acid in the paper becomes diluted and is washed out, and the parchment so formed is left a light or deep shade of yellow, according to the amount of dye used in the bath.

3. *Dye soluble in water but insoluble in acid.*—From one one-hundredth to ten ounces of Erie fast scarlet (color index No. 326) or some similar dye, depending on the shade desired, is ground up with a small amount of sulphuric acid from the parch-

mentizing bath, until a fine suspension of the dye in the acid is obtained. This is added to the parchmentizing bath so that the above amount is contained in one pound of parchmentizing acid. The paper is run through in the usual manner and washed in the usual way. As the water washes the acid out of the paper, the dye dissolves in it and thereby colors the "amyloid" which is formed at the same time.

4. *Dye soluble in water and in acid, but giving acid and water solutions which are different in color.*—The same procedure as described in Examples (1) or (2) is followed with a dye such as acid violet 4 B N S (color index No. 695) or some similar dye. Acid violet 4 B N S forms a yellow dye-bath with the sulphuric acid. The paper is put through the usual manner, and upon washing the yellow changes to violet, and the paper is dyed a shade of violet depending on the concentration of dye used in the acid.

5. *Dye insoluble in water but soluble or partially soluble in acid.*—The dye is dissolved in the acid or a suspension is made in the acid similarly as described in Example (3) in an amount equal to from one one-hundredth to ten ounces per pound of parchmentizing acid. Naphthylamine black D (color index No. 308) or some similar dye is used and the paper run through in the usual manner. Upon washing out the acid the dye is precipitated by the water and is firmly fixed in the "amyloid".

35 I am thus enabled also to produce, for the first time, parchmentized paper containing various dyestuffs which it has hitherto been impossible to use in the manufacture of such papers, namely, dyes which are not water-soluble. And, by this new method I am not only enabled to produce colored parchmentized papers in a greater variety of colors and shades, with less otherwise unavoidable loss of dyestuffs, and with more 40 satisfactorily constant and controllable effects, owing to the greater latitude in the choice of classes of dyes which may be employed in the manufacture of colored paper parchmentized by the methods described, 45 but I am also enabled thereby to produce colors not hitherto attainable with the hitherto known and applied methods.

In the first place, the old method of applying the dyestuff in the beaters required that 55 the coloring matter used be water-soluble. In addition to the disadvantage in the loss of coloring material by such process, this prescribed a limitation in the choice of dyestuffs, necessarily limiting the variety of colors and 60 shades. Furthermore, beyond the required quality of water-solubility, dyestuffs applied in the beaters must also be "basic" dyes in order that they would color the fiber of the paper as it has not been considered competent to use any mordant in a paper which was

to undergo the parchmentizing treatment in the acid bath. Makers of such paper were therefore limited substantially to water-soluble basic dyes for the purpose of dyeing of the paper by the process of coloring in the beaters. The process of coloring the paper after its formation and before parchmentizing by impressing or imprinting the dyestuff upon the paper by rollers carrying such colors is also limited to water-soluble dyes.

If any kind of a uniform color was to be expected such colors had to be insoluble in acid because otherwise the color impressed upon the paper from the rollers would again be dissolved off by the acid bath.

By being able to apply more varieties and classes of dyes which I have found can be used directly in the acid parchmentizing bath, I develop not only a superior product, but am enabled to make new grades of such paper incorporating dyes of a character which have never been used for the purpose. All of the limited numbers of dyes hitherto employed can also be used in my process, while with all the additional dyestuffs which I am enabled to use I can produce colored parchmentized papers of colors and shades heretofore not known in the art. Especially I am enabled to produce a black parchmentized paper of deep shade which it has not been possible to do satisfactorily by the old processes. It will also be evident, from the foregoing explanations and examples, that appropriate mixtures and combinations of colors may be made to produce numerous tints and shades in parchmentized paper hitherto entirely unknown in this art.

One of the advantages of my method of coloring these papers is that it permits closely coordinated control. After experiment has once determined just what mixtures and proportions are to be employed in order to produce any specialized color, shade, or tint, it is a relatively simple matter to so control the acid bath that it will be at all times of substantially the same composition, and the finished paper can be produced always in close approximation of the selected standard of color or tint.

Sulphuric or other acids or materials have been used in parchmentizing baths, but the former is preferably employed because of its greater availability and relative cheapness. I have therefore described my process of incorporating the colors in the parchmentizing bath as set forth in the specific illustrative examples in terms relating more specifically to the use of sulphuric acid; but it will be obvious to the paper-colorist chemist that by proper adjustment of the conditions to variations in solubilities and reactions substantially the same general treatments with necessary modifications can easily be determined by simple experiment and applied in sub-

stantially the same manner as herein set forth.

It is also obvious from the description of the process herein set forth that it is possible to make considerable variation in quantity and qualities of the dyes used according to the colors, shades, or general effects which it is desired to produce, without departing from the nature and scope of my invention, 10 and I wish to have it understood that the examples given in this specification have been embodied for the purpose of illustration, and not by way of limitation.

What I claim as new, and for which I pray 15 the issuance of Letters Patent, is:

1. In the art of manufacturing colored or tinted parchmentized paper, the process of passing the formed paper through an acid bath in which is dissolved dyestuff, and subsequently passing the paper so treated 20 through a water bath to dissolve or wash out the acid still present.

2. In the art of manufacturing parchmentized paper of the character described, a step 25 in the process, comprising the treatment of the paper with an acid bath in which dyestuff is dissolved.

3. In the art of manufacturing parchmentized paper of the character described, a step 30 in the process comprising the treatment of the paper with a parchmentizing bath in which dyestuff is dissolved.

4. In the art of manufacturing parchmentized paper of the character described, a step 35 in the process, comprising the treatment of the formed paper by immersing the same in a parchmentizing bath in which organic dyestuff is dissolved.

5. A parchmentized paper incorporating 40 dyestuffs soluble in acid but not soluble in water.

6. Parchmentized paper incorporating naphthylamine black D (color index No. 308).

7. In the process of parchmentizing paper, 45 the addition of dyestuffs to an acid parchmentizing bath.

8. In the process of manufacturing colored or tinted parchmentized paper which embraces a step consisting in treating such paper in an acid bath, the addition of the dyestuff to said acid bath.

9. In the process of manufacturing colored or tinted parchmentized paper which embraces a treatment of such paper in an acid parchmentizing bath, a step consisting of the addition to said bath of dyestuff which will not be destroyed by the acid of the bath.

10. In the art of manufacturing colored or 50 tinted parchmentized paper, the process of passing the formed paper through an acid bath in which is dissolved coal-tar dye-stuff, and subsequently passing the paper so treated through a water bath to dissolve or wash 55 out the acid still present.

11. Parchmentized paper which has incorporated therein a black organic acid-soluble water-insoluble dye.

12. Parchmentized paper incorporating acid-soluble water-insoluble organic dye- 70 stuff.

13. Parchmentized paper incorporating dye-stuff soluble in sulphuric acid and insoluble in water.

ROBERT IRVING COWEN.

75

80

85

90

95

100

105

110

115

120

125

130